

## UNITED STATES PATENT OFFICE

1,933,319

## ELECTROPLATING TANTALUM

Frank H. Driggs, Bloomfield, and William C. Lilliendahl, Montclair, N. J., assignors to Westinghouse Lamp Company, a corporation of Pennsylvania

No Drawing. Application July 26, 1930  
Serial No. 471,081

5 Claims. (Cl. 204—19)

This invention relates to the preparation of metals and more particularly to the preparation of rare refractory metals by the electrolytic decomposition of rare refractory metal compounds 5 in fused baths.

In copending application Serial No. 275,264 filed May 4, 1928 and entitled "Method of producing tantalum and other rare refractory metals by electrolysis of fused compounds," there is disclosed a method of producing tantalum metal powder by the electrolytic decomposition of a fused bath comprised of alkali metal halides containing a proportion of a double alkali metal tantalum halide compound. The tantalum metal 10 powder thus prepared is recovered from the fusion mixture by lixiviation methods and subjected to a vacuum sintering process to render the same coherent. The coherent tantalum metal thus obtained is substantially pure and may be readily 15 worked down into articles such as wire, rod, sheet, filament and the like.

Heretofore in the arts tantalum has been applied to many uses. Because of its chemical inertness and high melting point it has been proposed as a substitute for platinum in crucibles 20 and similar chemical ware.

In electric discharge devices, such as electron discharge devices of the evacuated type, gaseous conduction devices, radio tubes, X-ray tubes, incandescent lamps and the like it has been proposed to employ tantalum as electrode material, gas clean up agent, filament and the like. The successful application of tantalum as an electrode or as a gas clean up agent and filament is 35 restricted, however, by reason of the fact that the tantalum lacks the rigidity which is characteristic of the refractory metals, tungsten and molybdenum, for example. The physical characteristics of tantalum which permit its ready 40 mechanical deformation to desired shapes and sizes limit the application of the same in the arts.

It is one of the objects of the present invention to facilitate the use and application of tantalum in the arts.

It is another object of this invention to provide tantalum surfaced materials which are useful in the arts.

It is another object of this invention to provide 50 a process for electroplating tantalum upon metal surfaces.

Other objects and advantages will become apparent as the invention is more fully disclosed.

In copending application Serial No. 275,264 55 above identified there is disclosed a process for

depositing tantalum metal powder upon a cathode. In the practice of the invention set forth in this copending application it was one of the objects to prepare the tantalum in a reasonably coarse state, loosely adherent to the 60 cathode so that the same may be subsequently removed therefrom by mechanical means, such as scraping. In order to obtain this type of deposit upon the cathode current densities ranging from 0.5 to 1.0 amperes per  $\text{cm}^2$  (50-100 amperes 65 per decimeter<sup>2</sup>) were employed.

We have found that when current densities of a much lower order are employed that the tantalum thus deposited may be made to adhere to the cathode surface to form a smooth continuous 70 film thereon which is substantially impervious to acids and to gases.

As a specific example of the present invention we form an electroplated tantalum coating upon iron, nickel, molybdenum, tungsten and the like 75 surfaces in the following manner:

A fusion mixture comprising potassium chloride, potassium fluoride, potassium tantalum fluoride and tantalum oxide in the following relative proportion is employed: 80

|           |                                 |
|-----------|---------------------------------|
| 300 grams | KCl                             |
| 120 grams | KF                              |
| 100 grams | K <sub>2</sub> TaF <sub>7</sub> |
| 25 grams  | Ta <sub>2</sub> O <sub>5</sub>  |

This fusion mixture is placed in a graphite crucible and brought to fusion by any convenient means. The approximate melting point of this bath is 700 to 750° C. The bath is maintained during electrolysis at a temperature approximating 750° C. The base metal to be surfaced with the tantalum is immersed in the fused bath and allowed to remain therein until it has attained approximately the same temperature as the bath. Due to the corrosive action of the fusion mixture 95 the surface of the immersed metal will be substantially cleansed of all deleterious oxides. It is better, however, to subject the metal prior to immersion to the usual surface cleansing processes, such as subjecting the metal body to the 100 action of a reducing gas such as hydrogen, etching the surface with acid or alkali solutions or sand blasting. The latter method is to be preferred as the roughened surface materially facilitates the retention of the deposited tantalum 105 thereon.

The metal base thus prepared and immersed in the bath is given a final cleansing by making the same temporarily the anode in the bath so as to subject the same to anodic solution effects and 110

then is made the cathode. A current density of approximately .01 to 0.1 amperes per  $\text{cm}^2$  (1 to 10 amperes per decimeter<sup>2</sup>) is employed in effecting electro-plating of tantalum to the base metal.

5 The specific current density employed will vary materially with the different base metals being plated as will also the time interval necessary to effect a reasonably good deposit.

As an illustration reference should be made to 10 the following table wherein is given some representative current densities employed in the surfacing of nickel, iron and molybdenum articles with tantalum.

| 15 | Base metal | cm <sup>2</sup> in bath | Amp. per cm <sup>2</sup> | Time | Ampere minutes per cm <sup>2</sup> | Type of coating |
|----|------------|-------------------------|--------------------------|------|------------------------------------|-----------------|
| 20 | Ni.....    | 14                      | .217                     | 15   | 3.0                                | Too coarse      |
|    | Ni.....    | 10                      | .06                      | 10   | .5                                 | Good            |
|    | Ni.....    | 12                      | .041                     | 15   | .62                                | Best            |
| 30 | Fe.....    | 8                       | .062                     | 30   | 1.8                                | Good            |
| 40 | Mo.....    | 18                      | .028                     | 55   | 1.5                                | Good            |

25 The above table illustrates the type of coating obtained in the plating of strips of sheet metal with different current densities. In the plating of shaped articles, such as crucibles, radio tube plate (or anode electrodes) or the surfacing of lengths of wire, filament and the like, variations 30 in the current densities that may be employed and in the arrangement of elements within the bath must be made.

35 In the surfacing of a crucible, for example, the anode electrode must be shaped in the approximate convolution of the crucible. In the surfacing of a radio tube plate electrode it is preferable to electroplate the surface of a sheet of the base metal, such as nickel or molybdenum and thereafter shape the electrode therefrom. In the 40 surfacing of wire, filament and the like it is preferable to do the same in a continuous manner providing means exterior to the bath for cleansing the filament prior to entering the bath, said means depending primarily upon the nature of 45 the base filament employed.

50 The type of coating obtained by the practice of the above identified process can best be ascertained by immersing the coated metal in hot dilute nitric acid for an interval of time sufficient to indicate whether the base element is being attacked by the acid. The tantalum is not touched by this acid.

55 We have found that when a nickel or iron sheet or crucible shaped article has been so surfaced with tantalum that the article may be incandescent to relatively high temperatures in the open air without substantial oxidation or deterioration. The articles also may be subjected to

the action of acids without attack thereby, hydrofluoric acid alone being excepted.

Having broadly and specifically set forth the nature of the present invention it is apparent that there may be many modifications of the specific embodiment herein disclosed without departing essentially from the nature and scope of the invention as set forth in the accompanying claims, and that there may be many applications made of the electroplating process in the preparation of tantalum surfaced metal articles.

80

81

What is claimed is:

1. The method of forming a continuous adherent electro-plated tantalum surface upon an electrically conductive body comprising immersing said body in a fused bath comprised of alkali halide compounds containing a proportion of an ionized tantalum compound and electrolytically depositing the tantalum thereon at relatively low current densities ranging from 1 to 10 amperes per square decimeter. 90

2. The method of electrolytically depositing an adherent coating of tantalum upon an electrically conductive body comprising immersing said body in a fused bath comprised of alkali halide compounds containing a proportion of an ionized tantalum compound and electrolytically depositing the tantalum thereon at relatively low current densities ranging from 1 to 10 amperes per square decimeter. 100

3. The method of electroplating an adherent continuous tantalum film comprising immersing an electrically conducting body in a fused bath comprised of alkali halide compounds, a proportion of a double alkali metal-tantalum fluoride compound, and electrolytically depositing the tantalum on said body at relatively low current densities ranging from 1 to 10 amperes per square decimeter. 105

4. The method of electroplating an adherent continuous tantalum film comprising immersing an electrically conducting body in a fused bath comprised of potassium chloride and potassium fluoride compounds, a proportion of potassium tantalum fluoride and a proportion of tantalum oxide, and electrolytically depositing the tantalum on said body at cathode current densities ranging from 1.0 to 10.0 amperes per square decimeter. 110

5. As an article of manufacture, an electrically conductive body surfaced at least in part with a relatively smooth, continuous film of electrolytically deposited tantalum, said film being in the form of an even coherent layer which is firmly adherent to the conductive body. 125

130

FRANK H. DRIGGS.  
WILLIAM C. LILLIENDAHL.

60

134

65

140

70

145

75

150